

# United States Patent [19]

Krauss et al.

[11] Patent Number: 4,793,870

[45] Date of Patent: Dec. 27, 1988

- [54] **CONTINUOUS TREATMENT OF COLD-ROLLED CARBON HIGH MANGANESE STEEL**
- [75] Inventors: George Krauss, Evergreen, Colo.; Philip M. Roberts, Naperville, Ill.
- [73] Assignee: Signode Corporation, Glenview, Ill.
- [21] Appl. No.: 37,186
- [22] Filed: Apr. 10, 1987
- [51] Int. Cl.<sup>4</sup> ..... C21D 8/04
- [52] U.S. Cl. ..... 148/12.1; 148/12 F; 148/15; 148/154
- [58] Field of Search ..... 148/134, 14, 15, 156, 148/150, 154, 12 F, 12.1

[56] References Cited

U.S. PATENT DOCUMENTS

- 1,561,577 11/1925 Trautman ..... 134/122 R  
 1,561,578 11/1925 Trautman ..... 373/128  
 1,561,579 11/1925 Trautman ..... 148/15  
 1,700,002 1/1929 Trautman ..... 373/119  
 1,810,612 6/1931 Kathner ..... 148/156  
 1,937,420 11/1933 Wood et al. ..... 219/11  
 2,019,555 11/1935 Wood et al. ..... 219/11  
 2,164,850 7/1939 Wood et al. ..... 148/4  
 2,224,998 12/1940 Wood et al. ..... 148/10  
 2,300,329 10/1942 Wood et al. ..... 148/10  
 2,304,225 12/1942 Wood et al. ..... 219/11  
 2,345,181 3/1944 Cooper et al. ..... 13/25  
 2,462,202 2/1949 Kniveton ..... 148/13  
 2,716,079 8/1955 Wick et al. ..... 148/10  
 2,832,709 4/1958 Sendzimir ..... 148/13  
 2,864,607 12/1958 Renkin ..... 266/3  
 2,892,744 6/1959 Myers ..... 148/16  
 3,163,566 12/1964 Jenkins et al. ..... 148/150  
 3,181,977 5/1965 Sturgeon ..... 148/13.1  
 3,235,416 2/1966 Jenkins ..... 148/129  
 3,239,201 3/1966 Simich et al. ..... 266/3  
 3,277,270 10/1966 Trautman ..... 219/155  
 3,421,951 1/1969 Shelton ..... 148/39  
 3,615,926 10/1971 Taylor ..... 148/143

- 3,761,323 9/1973 Hunt et al. ..... 148/12  
 3,902,927 9/1975 Pernstal ..... 148/12  
 3,951,696 4/1976 Gondo et al. ..... 148/12  
 4,050,959 9/1977 Nakaoka et al. ..... 148/12.3  
 4,159,218 1/1979 Chatfield et al. ..... 148/12  
 4,243,441 1/1981 Wilson ..... 148/128  
 4,336,080 6/1982 Nakaoka et al. ..... 148/12  
 4,363,472 12/1982 Shimoyama et al. ..... 266/111  
 4,394,186 7/1983 Furukawa et al. ..... 148/12  
 4,407,680 10/1983 Gladman et al. ..... 148/12  
 4,436,561 3/1984 Takahashi et al. ..... 148/12  
 4,440,583 4/1984 Ikegami et al. ..... 148/128  
 4,448,614 5/1984 Morimoto et al. ..... 148/12.1

FOREIGN PATENT DOCUMENTS

1608163 10/1973 Fed. Rep. of Germany .

OTHER PUBLICATIONS

McGannon, H. E., ed., Making, Shaping and Treating of Steel, 9th ed., ©1971, pp. 1121-1125.

S. F. Radtke, Cosmos Engineering Inc. (USA).

Paulus et al, Study of the Heat Buckling and Shape Problems in Continuous Heat Treating Lines and Discussion of Proposed Solutions, pp. 424-439.

Inland Steel, MartInsite®, Ultra High Strength for Today's Needs, pp. 1-10.

High Strength, Low Alloy Steel—SAE J410, Jun. 1984, pp. 1.86-1.88.

Primary Examiner—Christopher W. Brody  
 Attorney, Agent, or Firm—Wood, Herron & Evans

[57] ABSTRACT

Cold-rolled, non-microalloyed carbon manganese steel (0.11% to 0.18% C, 1.20% to 1.40% Mn) is preheated at 700° to 1000° F., heated to 1500° to 1575° F., and quenched to 800° to 950° F. in a continuous process to develop minimum yield strength of 70,000 psi, minimum tensile strength of 85,000 psi, and 14% minimum elongation.

7 Claims, 2 Drawing Sheets





FIG. 1

U.S. Patent

Dec. 27, 1988

Sheet 2 of 2

4,793,870



FIG.2

## CONTINUOUS TREATMENT OF COLD-ROLLED CARBON HIGH MANGANESE STEEL

### BACKGROUND OF THE INVENTION

There exists today a group of steels which are characterized by among other things enhanced mechanical properties including higher yield strengths and tensile strengths than plain carbon structural steels. These are known as high-strength, low-alloy (HSLA) steels. Different types of HSLA steels are available, some of which are carbon-manganese steels and others of which are microalloyed by additions of such elements as niobium, vanadium, and titanium to achieve enhanced mechanical properties. The original demand for HSLA steels arose from the need to obtain improved strength-to-weight ratios to reduce dead weight in transportation equipment. In addition to the original uses, HSLA steels are used today in a wide range of applications including vehicles, construction machinery, materials-handling equipment, bridges and buildings.

Commercial HSLA steels typically have minimum yield strengths of 40 to 50 ksi and minimum tensile strengths of 60 to 70 ksi. The mechanical properties and other characteristics of HSLA steels are set forth in standard specifications such as SAE J410c. Microalloyed HSLA steels have even higher strengths on the order of minimum yield strengths of 50 to 80 ksi and minimum tensile strengths of 65 to 95 ksi. These steels use additions of alloying elements such as niobium, vanadium, titanium, zirconium and rare earth elements in concentrations generally below 0.10 to 0.15% to achieve higher strength levels. Heat treatment is not involved because the properties of microalloyed HSLA steels result from controlled rolling on continuous hot strip mills.

One grade of microalloyed, high-strength, low-alloy steel under SAE J410c is grade 970X, which is characterized by a minimum yield strength (0.2% offset) of 70,000 psi, minimum tensile strength of 85,000 psi, and minimum elongation (2-inch specimen) of 14%. As stated, this material exhibits its mechanical properties as hot rolled. When later cold reduced to sheet thickness, these steels are subjected to a low temperature recovery anneal for an extended period of time to maintain the controlled rolled mechanical properties. In addition to the increased cost because of the addition of microalloying elements, this recovery anneal is disadvantageous because of either the extended times required for box annealing or the enormous investment required for equipment for continuous annealing.

There thus exists today a need for steels possessing the desired combination of strength and ductility required for HSLA steel applications but which can be produced economically from cold reduced sheet stock without the need for extended recovery annealing. Moreover, there exists a need for such steels wherein the higher mechanical properties, particularly yield strength and tensile strength, are achieved without the intentional inclusion of microalloying agents such as niobium, titanium and vanadium, which otherwise would add significantly to the cost of the steel.

### SUMMARY OF THE INVENTION

It is among the principal objectives of this invention to provide a method for treating cold reduced steel compositions characterized by a relatively low carbon content and the absence of expensive microalloying

agents which nevertheless exhibit in the treated condition mechanical properties, i.e., yield strength, tensile strength, and elongation, meeting the specifications for microalloyed HSLA steels, for example, grade 970X of SAE J410c. Moreover, it is among the principal objectives of this invention to provide such a method for producing cold reduced steels having the uniformly higher mechanical properties of the microalloyed HSLA steels which can be produced in a continuous process at relatively high speed and very economically.

To these ends, the present invention is directed to a non-microalloyed low carbon, high manganese steel composition and to a heat treatment method therefor. The steel compositions included within this invention have a carbon content ranging from 0.11 to 0.18% by weight carbon and 1.20 to 1.40% by weight manganese. Microalloying elements such as niobium, titanium and vanadium are not added to the steel composition to achieve enhanced mechanical properties. The steel, which is cold reduced to a desired sheet thickness, e.g., in the range of 0.020 to 0.060 inch, is passed continuously through three heating stages. The first stage is a preheating stage wherein the temperature of the cold rolled sheet is raised to a temperature in the range of about 700° F. to 1000° F. The steel is then heated to a temperature in the range of 1500° F. to 1575° F., quenched at a temperature in the range 850° F. to 950° F., and then cooled to room temperature.

The heat treatment is carried out continuously at a line speed in the range of 50 to 300 feet/minute whereby a continuous length of steel strip of desired gauge and width is passed continuously and sequentially through the three heating stages.

One presently preferred steel composition is a steel having about 0.11 to 0.18% by weight carbon and about 1.20 to 1.40% by weight manganese, the balance being iron and the normal residuals from deoxidation. When treated in accordance with the heat treatment schedule described above, the treated steel exceeds the minimum yield strength of 70,000 psi, minimum tensile strength of 85,000 psi, and minimum elongation of 14% specified for grade 970X SAE J410c specifications.

The method of this invention for treating steels having the relatively low carbon and the manganese content recited and the absence of microalloying agents results in a cold reduced product having mechanical properties meeting or exceeding some existing HSLA steel specifications for microalloy steels. The present invention is thus characterized by the higher mechanical properties of some of the commercial microalloyed high-strength low-alloy steels but obtainable in a non-microalloyed, cold reduced low carbon steel and by the economies inherent in the absence of microalloying agents, and the continuous process for the treatment of a cold reduced product.

### BRIEF DESCRIPTION OF THE DRAWINGS

FIG. 1 is a schematic illustration of the treatment process.

FIG. 2 is a photomicrograph taken at 500x magnification of one steel composition treated by the method of this invention.

### DETAILED DESCRIPTION OF THE PREFERRED MODE

The carbon-manganese steel compositions treated by the method of this invention contain from about 0.11 to

0.18% by weight carbon and 1.20 to 1.40% by weight manganese. The steel is killed, preferably, aluminum killed and continuously cast, to achieve uniformity of mechanical properties. As a result, the composition can contain residual silicon and aluminum from the deoxidation process. The steel may also be a silicon killed or semi-killed steel.

Referring to FIG. 1, hot rolled coils of steel, which may be pickled and oiled, are cold reduced through a series of cold rolling passes to a sheet 10 having a desired reduced thickness, for example, on the order of 0.020 to 0.660 inch. The cold rolled and reduced sheet 10 is then passed over roller 11 and down into a preheat bath 12 which may be a bath of molten lead maintained at a temperature in the range of 700° to 1000° F. The lead bath may be heated by any of a number of means, e.g., natural gas or electricity. Alternatively to a lead bath, other media capable of providing a liquid bath having a temperature in the range of 700° to 1000° F. may be used. The material then passes upwardly out of the bath and over an elevated roller 14. The material then passes down into a second molten lead bath 16 which is the quench bath.

In the heating stage, the material is heated to a temperature in the range of 1500° to 1575° F. In the quench stage, the material is quenched at a temperature in the range of 800° to 950° F. Heating of the material in the heating stage is accomplished by resistance heating. That is, the preheat bath 12 and the quench bath 16 are maintained at a potential of about 90 volts and current of 8000 amperes with the quench bath being grounded. As a consequence, the sheet material 10 passing between the preheat bath and the quench bath shunts the current and is thereby resistance heated. The length of material passing through the heating stage, current, and travel speed are controlled to subject the material in the heating stage to the desired treatment temperature in the range of 1500° to 1575° F. A protective atmosphere is maintained in the heating stage by enveloping the sheet material 10 in an atmosphere housing 18 which is flushed with a protective exothermic gas. The gas prevents the sheet material from oxidizing as it passes from the preheat bath 12 to the quench bath 16. Alternatively to resistance heating, the material 10 may be heated by other heating means such as induction, infrared, and gas heating.

The quench bath 16 is also a lead bath which can be heated by such means as electric immersion heaters or radiant gas tubes to a temperature in the range of 800° to 950° F. After quenching, the material then passes out of the quench bath 16 and vertically upward over a roller 20 and through a charcoal chute 22 which contains ignited charcoal designed to prevent the lead from

known techniques, e.g., acid and/or abrasive cleaning, painting, plating, flattening, tension leveling, and the like.

The sheet material continuously passes through the preheat, heat and quench stages. Typical line speeds are on the order of 50 to 300 feet per minute. The preheat, heat, and quench stages are approximately 10 to 24 feet long. As a consequence, the material is heated or quenched very rapidly in each stage on the order of only 6-15 seconds, for example, at a line speed of 100 feet per minute.

Representative equipment for accomplishing such heating is disclosed in U.S. Pat. Nos. 2,224,988 and 2,304,225 to Wood et al. Again, heating and quenching media other than molten lead can be used for both the preheat and quench baths.

It is believed that the relatively short cycle times in the preheat, heat, and quench stages result in grain refinement and consequently increased strength. That is, in the preheat and heat stages, the strain introduced into the material from cold rolling causes recrystallization of the ferrite to a fine grain structure. The short cycle times limit grain growth keeping the grain size small, typically under 10 microns and frequently 3 to 4 microns and finer. In addition, small amounts of austenite form at the grain boundaries on heating and act to pin the grain boundaries against movement again serving to limit grain growth and resulting in higher strength levels. At the same time, the carbides in the pearlite are spheroidized and imperfections removed increasing the ductility of the steel. During the quench, the carbides precipitate introducing ductility and removing the potential for subsequent strain aging. The fine grained microstructure is illustrated by the photomicrograph in FIG. 2.

#### SPECIFIC EXAMPLES

Using the equipment described in FIG. 1, 2-inch wide by 0.044 inch thick steel strip cold reduced from 0.081 inch material was heat treated. The steel was aluminum killed for uniformity of properties and the composition contained 0.14% carbon, 1.33% manganese, 0.22% silicon and 0.019% aluminum, the silicon and aluminum components being residuals from the deoxidation of the steel before casting. The strip material traveled at a rate of 100 feet per minute. The length of the strip under the lead in the preheat bath was 10 feet, in the quench bath 20 feet, and in the heating stage 24 feet. Roller 14 was 8 feet above the lead baths. An optical pyrometer was used to measure strip temperature. The treatment schedule and resulting mechanical properties are set forth in Table I. A photomicrograph of the resulting microstructure is shown in FIG. 2.

TABLE I

| Sample Code | Preheat °F. | Strip Temp. °F. | Quench Temp. °F. | Tensile Strength (ksi) | Yield Strength (ksi) | % Elongation (2-inch gauge) | YS/TS | Hardness |
|-------------|-------------|-----------------|------------------|------------------------|----------------------|-----------------------------|-------|----------|
| 3-M         | 795         | 1535            | 855              | 92.7                   | 81.2                 | 18.7                        | .88   | 95       |
| 4-M         | 820         | 1500            | 950              | 86.0                   | 76.0                 | 22.0                        | .88   | 92       |

being dragged out of the quench bath on the sheet material. The sheet material which is now at a temperature of about 500° F. is then passed through a downstream water tank or water spray (not shown) to bring its temperature down to about 150° F. However, all of the transformation of the steel is completed by the time the material leaves the quench bath 16. After cooling, the material may be coiled for shipment or subsequently processed by known techniques or combination of

As may be seen from Table I, the mechanical properties resulting from the treatment process exceeded the minimum mechanical properties specified for grade 970X (70 ksi yield strength, 85 ksi tensile strength, 14% elongation). Both samples exhibited excellent ductility in combination with the higher strength levels.

The method of the present invention is applicable to a range of steel compositions within the compositional limits set forth above. As the preceding specific example shows, the treatment method provides low carbon high manganese cold reduced steels with the desired combination of strength and ductility characterizing commercial microalloyed and hot rolled high-strength low-alloy steels.

Thus having described the invention, what is claimed is:

1. A method of treating steel in a continuous process wherein the steel is cold reduced and has a composition of from about 0.11% to 0.18% by weight carbon and 1.20% to 1.40% by weight manganese, without the addition of microalloying agents for the purpose of achieving enhanced mechanical properties, comprising the steps of:

- (1) preheating the steel to a temperature in the range of 700° to 1000° F.;
  - (2) heating the steel to a temperature in the range of 1500° to 1575° F.; and
  - (3) quenching the steel at a temperature in the range of 800° to 950° F.;
- the treated steel having a minimum of 70,000 psi yield strength; 85,000 psi tensile strength; and 14% elongation.

2. A method for treating steel in a continuous process wherein the steel is cold reduced and has a composition of from about 0.14% by weight carbon and 1.33% by weight manganese, without the addition of microalloying agents for the purpose of achieving enhanced mechanical properties, comprising the steps of:

- (1) preheating the steel to a temperature in the range of 700° to 1000° F.;
  - (2) heating the steel to a temperature in the range of 1500° to 1575° F.; and
  - (3) quenching the steel at a temperature in the range of 800° to 950° F.;
- the treated steel having a minimum of 70,000 psi yield strength; 85,000 psi tensile strength; and 14% elongation.

3. A method of treating steel sheet and strip material in a continuous process wherein the steel material is cold reduced and has a composition of from about

0.11% to 0.18% by weight carbon and 1.20% to 1.40% by weight manganese, without the addition of microalloying agents for the purpose of achieving enhanced mechanical properties, comprising continuously passing the steel material through:

a molten lead bath held at a temperature in the range of 700° to 1000° F.;

a resistance heating stage wherein the material is heated to a temperature in the range of 1500° to 1575° F.; and

a molten lead bath held at a temperature in the range of 800° to 950° F.;

the treated material having a minimum of 70,000 psi yield strength; 85,000 psi tensile strength; and 14% elongation.

4. The method of claim 3 wherein the steel has a minimum of 75,000 psi yield strength; 85,000 psi tensile strength; and 16% elongation.

5. The method of claim 4 wherein the material has a cold reduced thickness in the range of about 0.020 to 0.060 inch.

6. The method of claim 3 wherein the material passes through the molten lead baths and the resistance heating stage each in less than about 15 seconds.

7. A method of treating steel sheet or strip material in a continuous process wherein the steel material is cold reduced aluminum killed steel having a composition of from about 0.11% to 0.18% by weight carbon and 1.20% to 1.40% by weight manganese, without the addition of microalloying agents for the purpose of achieving enhanced mechanical properties, comprising continuously passing the steel material through:

a preheating bath held at a temperature in the range of 700° to 1000° F.;

a resistance heating stage wherein the material is heated to a temperature in the range of 1500° to 1575° F.; and

a quenching bath held at a temperature in the range of 800° to 950° F.;

the treated material having a minimum of 70,000 psi yield strength; 85,000 psi tensile strength; and 14% elongation.

\* \* \* \* \*

UNITED STATES PATENT AND TRADEMARK OFFICE  
CERTIFICATE OF CORRECTION

PATENT NO. : 4,793,870

DATED : December 27, 1988

INVENTOR(S) : George Krauss et al

It is certified that error appears in the above-identified patent and that said Letters Patent is hereby corrected as shown below:

Column 1, line 52, "th" should be --the--.

Column 3, line 2, "mangnese" should be --manganese--.

Column 3, line 10, "roliing" should be --rolling--.

Column 3, line 12, "0.660" should be --0.060--.

Column 5, line 33, "he" should be --the--.

Signed and Sealed this

Nineteenth Day of September, 1989

Attest:

DONALD J. QUIGG

Attesting Officer

Commissioner of Patents and Trademarks